

## UNITED STATES PATENT OFFICE

2,340,881

COMPOSITION FOR LUBRICATING AND  
SOFTENING TEXTILE FIBERS

Maurice J. Kelley, Newark, and Edwin A. Robinson, Chatham, N. J., assignors to National Oil Products Company, Harrison, N. J., a corporation of New Jersey

No Drawing. Application August 22, 1939,  
Serial No. 291,342

21 Claims. (Cl. 252—8.8)

This invention relates to compositions suitable for lubricating and softening textiles, more specifically to textile lubricants and softeners comprising fatty acid amides.

It has previously been proposed to employ fatty acid amides such as oleic acid amide or oleic acid methyl amide for lubricating and softening textiles. However, since it has been found that organic softeners are most satisfactorily applied to textile material in the form of aqueous dispersions thereof, the low water dispersibility of these amides renders them somewhat disadvantageous for use in this connection. While it has been proposed to solubilize amides of polyamines by treatment with acids, it has been found that in many cases the solubilization accomplished by such treatment is not sufficient to enable these amides to be successfully applied to textiles in the form of aqueous dispersions thereof.

It has also been proposed to employ amides prepared by reacting monoethanolamine with fatty materials as textile lubricants and softeners; such amides, however, are also not as water-dispersible as might be desired. The use of textile lubricants and softeners comprising an amide of monoethanol triethylene tetramine has also been suggested; it has been found, however, that the employment of amides of this amine causes objectionable yellowing of the textile fibers after the fibers treated therewith have been permitted to stand for a short period of time.

From the above discussion it will be evident that while a large number of fatty acid amides of various types have been suggested for use as textile lubricants and softeners, substantially all of these amides have the disadvantage of either being relatively non-dispersible in water or of causing objectionable yellowing of the textile fiber after the fiber has been permitted to stand for a short period of time. Therefore, there has been a constant demand for lubricants and softeners in the textile industry which do not possess either of the above disadvantages. As yet, however, this demand has not been satisfied.

It is the object of this invention to prepare textile lubricants and softeners which may be readily applied to textile fibers in the form of aqueous dispersions thereof, and which do not cause objectionable yellowing of the textile material even after prolonged standing.

We have found that compositions comprising a certain class of fatty amides may be applied to textile materials in the form of aqueous dispersions thereof, whereby excellent softness, drape and pliability are imparted to the mate-

rial without causing any appreciable yellowing of the material even after prolonged standing. In accordance with our invention textile lubricants and softeners are employed which comprise a fatty amide having the general formula



in which  $R_1$  denotes a fatty acid radical containing more than 5 carbon atoms;  $R_2$  denotes an organic radical containing not more than 6 carbon atoms having an unsatisfied valence at both ends thereof and selected from the group consisting of straight chain hydrocarbon radicals, straight chain hydrocarbon radicals having a hydrogen atom replaced by a hydroxyl group, straight chain hydrocarbon radicals and straight chain hydrocarbon radicals having a hydrogen atom replaced by a hydroxyl group, which radicals contain an ether linkage, and straight chain hydrocarbon radicals containing a keto grouping;  $A$  denotes a radical containing not more than 22 carbon atoms and selected from the group consisting of hydrogen, alkyl radicals, alkylol radicals, acyl radicals, and alkyl and alkylol radicals containing an ether or thio ether linkage; and  $B$  denotes a radical containing not more than 22 carbon atoms and selected from the group consisting of alkyl radicals, alkylol radicals, acyl radicals, and alkyl and alkylol radicals containing an ether or thio ether linkage, at least one of said  $R_2$ ,  $A$  and  $B$  radicals containing at least one hydroxyl group. The amides of our invention may easily be dispersed in aqueous media and the dispersions applied to textile fibers so as to give an excellent feel to the fibers without causing objectionable yellowing of the fibers even after prolonged standing. The preferred products of our invention are those having the general formula  $R_1CONH-CH_2CH_2-NH-C_2H_4OH$ , since these products may be prepared from the readily available ethanol ethylene diamine, are readily dispersible in aqueous media and display particularly effective properties when employed as textile lubricants and softeners. We have found that in every case the amides of our invention give results which are far superior to those obtainable with any other amide softeners now on the market.

50 The amides of our invention may be prepared by reacting an amine having the general formula



55 in which  $R_2$ ,  $A$  and  $B$  are as above defined, at

least one of said R<sub>2</sub>, A and B radicals containing at least one hydroxyl group, with a fatty acid containing more than 5 carbon atoms or with a derivative thereof capable of reacting with amines to form amides. Thus, for example, the following amines have been found to be suitable for use in the preparation of the products of our invention: ethanol ethylene diamine, 1-amino 3 methyleneamino isopropanol, N-ethyl N-ethanol ethylene diamine, N,N diethanol ethylene diamine, isopropanol ethylene diamine, 1-amino 3-dimethylamino isopropanol, 1-amino 2-ethyl 3-methylamino isopropanol, 1-amino 2-ethyl 3-ethanol-amino isopropanol and 1-aminodimethyl 5-methylaminodimethyl n-pentanol-3. We prefer to employ ethanol ethylene diamine in the practice of our invention since this amine is readily available and furnishes excellent water-dispersible textile lubricants and softeners when treated with fatty acids or their derivatives. It is to be understood, however, that other amines having the above generic formula may also be employed in the practice of our invention.

The fatty compounds with which the above amines may be reacted in accordance with our invention may be any fatty acid having more than 5 carbon atoms or a derivative thereof capable of reacting with amines to yield amides. Thus, for example, fatty acids such as stearic acid, capric acid, oleic acid, coconut oil fatty acids or mixtures thereof, and fatty acid derivatives such as olive oil, coconut oil, cod oil, sperm oil, japan wax, methyl oleate and glycerol mono- or di-stearate may be employed to react with the amines. Naphthenic acids or their esters may also be reacted with amines of the above type to yield amides suitable for use in accordance with our invention, and we intend to include such reaction products within the scope of the term "fatty amides" since the properties of the naphthenic amides are entirely similar to the properties of the amides formed by reacting the amines with fatty acids or their derivatives. We have found that triglycerides of fatty acids containing more than 5 carbon atoms, e. g., coconut oil, teaseed oil, hydrogenated soy-bean oil and the like, react easily with the amines and yield amides having somewhat superior softening properties than those obtained by reacting the corresponding free fatty acids with the amines; hence we prefer to employ triglycerides of fatty acids having more than 5 carbon atoms as the fatty compounds reacted with the amines.

The reaction of the amine with the fatty compound may be carried out in any suitable manner. The amount of fatty compound employed per mol of amine will vary depending upon the nature of the fatty compound used; thus if a fatty acid is to be reacted with an amine, approximately equimolecular amounts of the acid and amine may be employed, whereas if a triglyceride such as coconut oil is used, approximately one-third of a mol of triglyceride per mol of amine may be employed. The temperature of the reaction may vary between about 100° C. and the boiling point of the amine, but preferably temperatures between about 125° C. and about 175° C. are employed. The reaction is preferably carried out at atmospheric pressure, but pressures below or above atmospheric may be used if desired. The reaction time may vary widely depending upon the particular ingredients employed; generally the reaction time will be between about 2 hours and about 48 hours. The products obtained from the reaction may be recovered in any suitable

manner, and, if necessary, purified before being used as textile lubricants and softeners.

The fatty amides of our invention may be applied to textile materials in any suitable manner. Because of the fact that these amides are dispersible in aqueous media, we have found it most advantageous to apply these amides to textile fabrics in the form of aqueous dispersions thereof. These dispersions may be prepared in a variety of ways. We have found that aqueous dispersions of the amides of our invention are most advantageously prepared by mixing the amide, preferably in liquid condition, with a dilute aqueous solution of an acid such as acetic acid, hydrochloric acid or lactic acid, whereby stable dispersions of the amides are formed immediately. These dispersions may contain any suitable amount of the fatty amide, but we prefer to employ dispersions containing between about 0.001% and about 5% thereof; thus it will be observed that dispersions containing very small amounts of the amides of our invention are capable of imparting an excellent finish to textile fabrics. In many cases it may be desirable to prepare relatively concentrated dispersions of the amide, e. g., dispersions containing 25% thereof, and then dilute the dispersions thus prepared to the desired concentration before use; this method of preparing the dispersions is advantageous when it is desired to store or ship the dispersions prior to use. Textile fabrics treated with the amides of our invention show no objectionable yellowing even after prolonged periods of time.

It is to be understood that while it is preferred to apply the amides of our invention to textile fabrics in the form of aqueous dispersions thereof, these amides may be applied in any other suitable manner without interfering with the excellent softness, pliability and drape which they impart to the fabrics.

The following examples are illustrative of our invention. Amounts are given in parts by weight.

#### Example I

45 233 parts of coconut oil and 104 parts of ethanol ethylene diamine were mixed and heated at a temperature of about 150° C. for about 12½ hours. A light cream colored solid product was obtained. This product was melted and hot water added thereto until an 0.015% dispersion of the amide was formed. Rayon fabric was then immersed in this dispersion for 10 minutes at a temperature of about 40° C. At the end of this time, the fabric was removed, squeeze-rolled, dried and ironed lightly. The fabric was found to have excellent softness and drape, and did not yellow even after prolonged standing.

#### Example II

60 680 parts of coconut oil and 156 parts of ethanol ethylene diamine were mixed and the mixture heated at a temperature between about 150° C. and about 170° C. for 12 hours. A light tan solid dispersible in water was obtained. This product was melted and hot water added thereto until an 0.015% dispersion of the amide was formed. This dispersion was then applied to rayon fabric as described in Example I, whereby a fabric was obtained having excellent softness and drape, and which did not yellow even after prolonged standing.

#### Example III

75 28 parts of oleic acid and 10 parts of ethanol ethylene diamine were mixed and heated at a temperature between about 150° C. and about

170° C. for 12 hours. The resulting product was melted and 175 parts of a warm 4% acetic acid solution were added thereto. This solution was then diluted until an 0.015% dispersion of the amide was formed and this dispersion applied to rayon fabric as described in Example I, whereby a fabric was obtained having excellent softness and drape, and which did not yellow even after prolonged standing.

*Example IV*

33 parts of castor oil and 10 parts of ethanol ethylene diamine were mixed and the mixture heated to a temperature between about 150° C. and about 170° C. for 8 hours, whereby a yellow liquid was obtained. This liquid was mixed with 205 parts of a hot 4% acetic acid solution, and the resulting solution diluted so as to form an 0.015% dispersion of the amide. This dispersion was applied to rayon fabric as described in Example I, whereby a fabric was obtained having excellent softness and drape, and which did not yellow even after prolonged standing.

*Example V*

74 parts of teaseed oil and 26 parts of ethanol ethylene diamine were mixed and the mixture heated at a temperature between about 150° C. and about 170° C. for 8 hours. The product was a light tan solid. This product was melted and 205 parts of a hot 4% acetic acid solution were added thereto. The resulting solution was diluted until an 0.015% dispersion of the amide was formed. This dispersion was applied to rayon fabric as described in Example I, whereby a fabric was obtained having excellent softness and drape, and which did not yellow even after prolonged standing.

*Example VI*

31 parts of hydrogenated soybean oil and 11 parts of ethanol ethylene diamine were mixed and the mixture heated at a temperature between about 150° C. and about 170° C. for 8 hours. The resulting solid was melted and 205 parts of a hot 4% acetic acid solution were added thereto. The solution thus obtained was then diluted until an 0.015% dispersion of the amide was formed. This dispersion was then applied to rayon fabric as described in Example I, whereby a fabric was obtained having excellent softness and drape, and which did not yellow even after prolonged standing.

It will be evident from the above description that our invention provides novel textile lubricants and softeners having properties which make them superior to lubricants and softeners heretofore employed. Therefore, our invention will be of great interest to those engaged in the finishing of textile materials.

The products of our invention may be further treated, if desired, to produce substances having desirable properties. For example, the amides may be sulfated or phosphated to yield wetting, dispersing and emulsifying agents, or they may be treated with acetic anhydride to yield products having excellent detergent and dispersing properties. Our novel products may also be treated in a variety of other manners known to the art so as to yield useful substances.

Since certain changes may be made in the above products and different embodiments of the invention could be made without departing from the scope thereof, it is intended that all matter contained in the above description shall be in-

terpreted as illustrative and not in a limiting sense.

Having described our invention, what we claim as new and desire to secure by Letters Patent is:

- 5 1. A composition of matter comprising an amide which is the condensation product of a hydroxy-alkylated polyamine with a glyceride containing only substantially saturated non-hydroxylated fatty radicals.
- 10 2. A composition of matter comprising an amide which is the condensation product of a polyamine of the type in which at least one of the amino groups contains a hydroxy-alkyl group, with a glyceride containing only substantially saturated non-hydroxylated fatty radicals.
- 15 3. A composition of matter comprising an amide which is the condensation product of monoethanol-ethylene-diamine with a glyceride containing only substantially saturated non-hydroxylated fatty radicals.
- 20 4. A composition of matter for lubricating and softening textile fibers comprising amides which are the condensation products of a hydroxy-alkylated polyamine with coconut oil glycerides.
- 25 5. A composition of matter for lubricating and softening textile fibers comprising amides which are the condensation products of a hydroxy-alkylated polyamine with hydrogenated soyabean oil glycerides.
- 30 6. A composition of matter comprising amides which are the condensation products of monoethanol-ethylene-diamide with coconut oil glycerides.
- 35 7. A composition of matter comprising amides which are the condensation products of monoethanol-ethylene-diamine with hydrogenated soyabean oil glycerides.
- 40 8. A composition of matter for lubricating and softening textile fibers consisting of an aqueous dispersion, in dilute acid solution, of an amide which is the condensation product of a hydroxy-alkylated polyamine with a glyceride containing only substantially non-hydroxylated fatty radicals.
- 45 9. A composition of matter for lubricating and softening textile fibers consisting of an aqueous dispersion, in dilute acid solution, of an amide which is the condensation product of a polyamine of the type in which at least one of the amino groups contains a hydroxy-alkyl group, with a glyceride containing only substantially non-hydroxylated fatty radicals.
- 50 10. A composition of matter for lubricating and softening textile fibers consisting of an aqueous dispersion, in dilute acid solution, of an amide which is the condensation product of monoethanol-ethylene-diamine with a glyceride containing only substantially non-hydroxylated fatty radicals.
- 55 11. Compositions of matter for lubricating and softening textile fibers consisting of aqueous dispersions, in dilute acid solutions, of amides which are the condensation products of a hydroxy-alkylated polyamine with coconut oil glycerides.
- 60 12. Compositions of matter for lubricating and softening textile fibers consisting of aqueous dispersions, in dilute acid solutions, of amides which are the condensation products of a hydroxy-alkylated polyamine with hydrogenated soyabean oil glycerides.
- 65 13. Compositions of matter for lubricating and softening textile fibers consisting of aqueous dispersions, in dilute acid solutions, of amides which are the condensation products of monethanol-ethylene-diamine with coconut oil glycerides.
- 70

14. Compositions of matter for lubricating and softening textile fibers consisting of aqueous dispersions, in dilute acid solutions, of amides which are the condensation products of monoethanol-ethylene-diamine with hydrogenated soya-bean oil glycerides.

15. A composition of matter consisting of an aqueous dispersion, in dilute acid solution, of an amide which is the condensation product of a hydroxy alkylated polyamine with a glyceride containing only substantially saturated, non-hydroxylated fatty radicals.

16. A composition of matter consisting of an aqueous dispersion, in dilute acid solution, of an amide which is the condensation product of a polyamine of the type in which at least one of the amino groups contains a hydroxy-alkyl group, with a glyceride containing only substantially saturated, non-hydroxylated fatty radicals.

17. A composition of matter consisting of an aqueous dispersion, in dilute acid solution, of an amide which is the condensation product of monoethanol-ethylene-diamine with a glyceride

containing only substantially saturated, non-hydroxylated fatty radicals.

18. Compositions of matter consisting of aqueous dispersions, in dilute acid solutions, of amides which are the condensation products of a hydroxy-alkylated polyamine with coconut oil glycerides.

19. Compositions of matter consisting of aqueous dispersions, in dilute acid solutions, of amides which are the condensation products of a hydroxy-alkylated polyamine with hydrogenated soyabean oil glycerides.

20. Compositions of matter consisting of aqueous dispersions, in dilute acid solutions, of amides which are the condensation products of monoethanol-ethylene-diamine with coconut oil glycerides.

21. Compositions of matter consisting of aqueous dispersions, in dilute acid solutions, of amides which are the condensation products of monoethanol-ethylene-diamine with hydrogenated soyabean oil glycerides.

MAURICE J. KELLEY.  
EDWIN A. ROBINSON.

CERTIFICATE OF CORRECTION.

Patent No. 2,340,881.

February 8, 1944.

MAURICE J. KELLEY, ET AL.

It is hereby certified that error appears in the printed specification of the above numbered patent requiring correction as follows: Page 3, first column, line 64, for "fosphated" read --phosphated--; and second column, line 32, claim 6, for "diamide" read --diamine--; lines 43, 51 and 58, claims 8, 9 and 10 respectively, after "substantially" insert --saturated--; and that the said Letters Patent should be read with this correction therein that the same may conform to the record of the case in the Patent Office.

Signed and sealed this 25th day of April, A. D. 1944.

Leslie Frazer

Acting Commissioner of Patents.

(Seal)

CERTIFICATE OF CORRECTION.

Patent No. 2,340,881.

February 8, 1944.

MAURICE J. KELLEY, ET AL.

It is hereby certified that error appears in the printed specification of the above numbered patent requiring correction as follows: Page 3, first column, line 64, for "fosphated" read --phosphated--; and second column, line 32, claim 6, for "diamide" read --diamine--; lines 43, 51 and 58, claims 8, 9 and 10 respectively, after "substantially" insert --saturated--; and that the said Letters Patent should be read with this correction therein that the same may conform to the record of the case in the Patent Office.

Signed and sealed this 25th day of April, A. D. 1944.

Leslie Frazer

(Seal)

Acting Commissioner of Patents.